

[54] **ALKALI FREE LEAD SILICATE GLASS  
MEDIUM FOR ULTRASONIC DELAY LINES**

[76] Inventors: **Takahiro Inamura; Kenichi  
Sawamoto; Nobukazu Niizeki**, all of  
Laboratory of Nippon Telegraphy &  
Telephone Public Corporation,  
9-11, 3-chome, Midori-cho;  
**Munehisa Tsunekawa; Yasuyuki  
Nakata**, both of Ohi Kogyo of  
Nippon Kogaku K.K., 6-3, 1-chome,  
Nishi-Ohi, all of Tokyo, Japan

[22] Filed: June 19, 1972

[21] Appl. No.: 264,338

**Related U.S. Application Data**

[63] Continuation-in-part of Ser. No. 63,194, Aug. 11,  
1970, abandoned.

[52] **U.S. Cl.** ..... 106/53

[51] **Int. Cl.** ..... C03c 3/10, C03c 3/30, C03c 3/04

[58] **Field of Search** ..... 106/53

[56]

**References Cited**

**UNITED STATES PATENTS**

3,598,619 8/1971 Mikoda et al..... 106/53

**FOREIGN PATENTS OR APPLICATIONS**

1,118,422 7/1968 Great Britain ..... 106/53

2,005,676 12/1969 France ..... 106/53

4,223,949 11/1967 Japan ..... 106/53

*Primary Examiner*—Winston A. Douglas

*Assistant Examiner*—Mark Bell

*Attorney, Agent, or Firm*—Shapiro and Shapiro

[57]

**ABSTRACT**

A glass medium suitable for ultrasonic delay lines employs a composition which consists essentially of 36 to 46 percent of  $\text{SiO}_2$ , 35 to 60 percent of  $\text{PbO}$ , 0 to 20 percent of  $\text{AlF}_3$  and 0 to 10 percent of  $\text{BaF}_2$ , the total content of the  $\text{AlF}_3$  and  $\text{BaF}_2$  being present in a range of 2 to 20 percent, the percentage being by weight.

**4 Claims, 4 Drawing Figures**

FIG. 1



FIG. 2



FIG. 3



FIG. 4



## ALKALI FREE LEAD SILICATE GLASS MEDIUM FOR ULTRASONIC DELAY LINES

This application is a continuation-in-part of our pending application Ser. No. 63,194; filed Aug. 11, 1970, now abandoned.

### FIELD OF INVENTION

The present invention relates to a glass medium for ultrasonic delay lines having improved acoustic properties.

### BACKGROUND OF INVENTION

In general, an ultrasonic delay line consists of a medium through which acoustic waves are propagated, an input transducer fixed to a suitable portion of the medium for converting electrical signals into mechanical signals and an output transducer for converting the mechanical signals again into electrical signals.

The most important factors of a medium used as a delay line are that the delay time will not be varied by temperature variation, that the attenuation of the propagated acoustic wave be minimal, and that the aging also be minimal. Glasses as ultrasonic media are required to meet severe conditions for such special uses. For example, when a glass is used as a delay line in a PAL color television receiver, the variation in delay time together with the aging must be within  $\pm 80$  ppm. The attenuation is preferred to be less than  $10 \times 10^{-3}$  db/cycle when measured with a frequency higher than 1 MHz. A fused silica which has been used widely as a delay line has a temperature coefficient (a ratio of variation of delay time to a temperature rise of 1°C) of about 80 ppm/°C. The glasses available on the market have a temperature coefficient from 10 ppm/°C to 50 ppm/°C and an aging from 100 ppm to 1,000 ppm, which depending upon their compositions represent a wide variation. Conventional glasses do not possess the properties to permit their satisfactory use as delay lines.

### SUMMARY OF INVENTION

It is therefore the primary object of the present invention to provide a glass composition to be used as a delay line which eliminates the defects encountered with prior art glass compositions, and which possesses satisfactory properties as a delay line. The temperature coefficient is in the range of -5 to +5 ppm/°C, the attenuation is less than  $10 \times 10^{-3}$  db/cycle when measured with a frequency of 5 MHz, and the aging is almost zero. Another advantage resides in the fact that glass compositions in accordance with the present invention may be produced in a considerably shorter annealing time as compared to the time required to produce prior art delay line glass. As a result, aging is minimized.

Furthermore, the viscosity and the melting temperature of molten glass made in accordance with the invention are lower because the glass contains fluorides, whereby melting and forming of the glass are greatly facilitated.

In summary, the novel features which are believed to characterize the present invention reside in the facts that the glass compositions of the present invention possess every property to satisfy the conditions required as a delay line and that the production of the glass is much facilitated.

### BRIEF EXPLANATION OF THE DRAWING

FIG. 1 is a schematic illustration of a bar-shaped ultrasonic delay line;

FIG. 2 is a graph illustrating the composition of a glass in accordance with the present invention;

FIG. 3 is a graph illustrating rate of variation of delay time due to aging; and

FIG. 4 is a graph illustrating the rate of variation of delay time due to temperature variation.

### PREFERRED EMBODIMENTS OF THE INVENTION

The invention may be understood with reference to FIG. 1, which shows a common and simple form of delay line consisting of a delay line medium 2 in the form of a bar and input and output transducers 1 and 3 fixed to the ends thereof. The shear waves of the mechanical signals converted by the input transducer 1 propagate through the medium 2 and are converted again into the electrical signals by the output transducer 3. The delay time is the time for the acoustic wave to propagate through the medium 2 between the input and output transducers 1 and 3.

FIG. 2 is a graph illustrating the composition range of a glass composition in accordance with the present invention. The glass consists of 36 - 46 percent by weight of  $\text{SiO}_2$ , 35 - 60 percent by weight of  $\text{PbO}$ , 0 - 20 percent by weight of  $\text{AlF}_3$  and 0 - 10 percent by weight of  $\text{BaF}_2$ . The total content of the  $\text{AlF}_3$  and  $\text{BaF}_2$  is present in the range of 2 to 20 percent by weight. When the fluoride content is smaller than the above mentioned range, the viscosity of the fused glass is increased, and unresolved  $\text{SiO}_2$  tends to remain so that it is difficult to attain a high degree of homogenization. It is therefore preferable that the fluoride content be higher than 2 percent by weight. From the standpoint of stability, the fluoride content is preferably less than 20 percent by weight. The contents of  $\text{PbO}$  and  $\text{SiO}_2$  are somewhat different depending upon the contents and types of fluorides, but a glass having a temperature coefficient in the range of -5 to +5 ppm/°C may be obtained by the contents of 36 - 46 percent by weight of  $\text{SiO}_2$  and 35 - 60 percent by weight of  $\text{PbO}$ . The attenuation of the glass of the invention is less than  $10 \times 10^{-3}$  db/cycle when measured with a frequency higher than 1 MHz, and the aging of delay time is less than 50 ppm by an accelerated aging test in which the glass is subjected to a strain of  $10^{-6}$  at 40°C with an alternating current of 1 MHz.

Since the glass of this invention contains a lead oxide, the velocity of shear wave may be small so that the dimensions of the glass may be made smaller compared with the prior art glass.

The table below shows the compositions, of the Examples and their acoustic characteristics:

| Examples                  | 1    | 2    | 3    | 4    | 5    | 6    | 7    | 8    | 9    |
|---------------------------|------|------|------|------|------|------|------|------|------|
| $\text{SiO}_2$ (% by wt.) | 40.0 | 40.0 | 40.5 | 40.0 | 41.0 | 41.0 | 43.3 | 38.0 | 42.0 |
| $\text{PbO}$              | 56.0 | 53.5 | 51.0 | 49.5 | 48.5 | 50.5 | 45.9 | 48.0 | 40.0 |
| $\text{AlF}_3$            | 4.0  | 6.5  | 8.5  | 10.5 | 10.5 |      | 2.8  | 10.5 | 11.5 |
| $\text{BaF}_2$            |      |      |      |      |      | 8.5  | 8.0  | 3.5  | 6.5  |

Table—Continued

| Examples                                                                                     | 1    | 2    | 3    | 4    | 5    | 6    | 7    | 8    | 9    |
|----------------------------------------------------------------------------------------------|------|------|------|------|------|------|------|------|------|
| Temperature coefficient ppm/ $^{\circ}\text{C}$ 0 $^{\circ}\text{C}$ – 50 $^{\circ}\text{C}$ | 0.3  | 0.5  | 1.3  | 1.0  | 2.6  | 2.0  | 5.0  | 4.8  | 0.8  |
| Velocity km/sec.                                                                             | 2.51 | 2.56 | 2.60 | 2.63 | 2.64 | 2.50 | 2.61 | 2.63 | 2.71 |

The attenuation of each of the Examples was less than  $10 \times 10^{-3}$  db/cycle and the aging in 20 years was less than 50 ppm as shown in FIG. 3. The temperature variations for Examples 1 and 3 are shown in FIG. 4. Aging tests were made at 50 $^{\circ}\text{C}$  under a continuous strain of  $10^{-6}$  by an alternating current of 5MHz. The density of each glass was about 4g/cm<sup>3</sup>.

In the production of prior art glasses for delay lines, fine control of temperature and time are required. In accordance with the present invention control of temperature and time are not critical and the acoustic properties of the glass of the present invention will not vary though the control of conditions of temperature and time may vary. For example, in case of Example 1 consisting of 40.0 percent by weight of SiO<sub>2</sub>, 56.0 percent by weight of PbO and 4.0 percent by weight of AlF<sub>3</sub>, the temperature coefficient, attenuation and aging remained almost unchanged even when the annealing temperature was changed from 1 $^{\circ}\text{C}/\text{Hr.}$  to 30 $^{\circ}\text{C}/\text{Hr.}$ , with a decrease in velocity of only 0.5 percent. The viscosity of the molten glass of the invention is reduced because the glass contains fluorides. For example, the melting temperature of the glass of the invention is lower by 50° – 150 $^{\circ}\text{C}$  than the melting temperature of the prior art glass containing only oxides. Thus the glass melting conditions are much improved.

The raw materials of the glass in accordance with the present invention may be mixed in the conventional manner and melted in a clay pot or platinum crucible at a temperature from 1,200° to 1,350 $^{\circ}\text{C}$ . The fused glass may be formed by the conventional method. The continuous flow or tank furance method may, of course, be employed. When a refining agent such as Sb<sub>2</sub>O<sub>3</sub>, As<sub>2</sub>O<sub>3</sub>, etc., is added to the raw materials in a very small quantity, the homogenization of the glass may be much improved.

For example, glass in accordance with Example 1 is

10 prepared by the following process. A glass batch (total amount about 200.0 kg) comprising 80.0 kg of SiO<sub>2</sub>, 108.74 kg of PbO, 8.1 kg of AlF<sub>3</sub> and 1.0 kg of Sb<sub>2</sub>O<sub>3</sub> is well mixed by a known method, and the mixture is heated at 1,350 $^{\circ}\text{C}$  for 5 hours in a clay crucible. The molten glass is stirred for 15 minutes under 40 revolutions per minute. Then the molten mixture is cooled to a temperature suitable for casting. The cooled, molten glass is thrown in a cast, and annealed to room temperature at an annealing rate 1.5 $^{\circ}\text{C}/\text{hr.}$

15 20 Glass made in accordance with the present invention has satisfactory properties for ultrasonic delay lines and may be produced in a simple manner.

We claim:

25 30 35 40 45 1. A glass medium for ultrasonic line having the range of -5 to +5 ppm/ $^{\circ}\text{C}$  of the temperature coefficient of delay time, attenuation of less than approximately  $10 \times 10^{-3}$  db/cycle at a frequency higher than 1 MHz, and aging of delay time of less than 50 ppm, the glass medium being devoid of an alkali ion and consisting essentially of, by weight, 36 to 46 percent of SiO<sub>2</sub>, 35 to 60 percent of PbO, 0 to 20 percent of AlF<sub>3</sub> and 0 – 10 percent of BaF<sub>2</sub>, the total content of the AlF<sub>3</sub> and BaF<sub>2</sub> being present in a range of 2 to 20 percent.

2. A glass medium according to claim 1 wherein the SiO<sub>2</sub> is in the amount of 40.0 percent, the PbO is in the amount of 56.0 percent, and the fluoride is AlF<sub>3</sub> in the amount of 4.0 percent.

3. A glass medium according to claim 1, wherein the SiO<sub>2</sub> is in the amount of 40.0 percent, the PbO is in the amount of 53.5 percent, and the fluoride is AlF<sub>3</sub> in the amount of 6.5 percent.

4. A glass medium according to claim 1 wherein the SiO<sub>2</sub> is in the amount of 41.0 percent, the PbO is in the amount of 50.5 percent, and the fluoride is BaF<sub>2</sub> in the amount of 8.5 percent.

\* \* \* \* \*